

Aug. 26, 1930.

F. C. SIMMS

1,773,825

PYROMETER TUBE

Filed Nov. 4, 1927

*Fig. 1.*

11



*Fig. 2.*



INVENTOR

*Frank C. Simms.*

BY *N.M. Biebel*  
ATTORNEY

## UNITED STATES PATENT OFFICE

FRANK C. SIMMS, OF EAST PALESTINE, OHIO

## PYROMETER TUBE

Application filed November 4, 1927. Serial No. 230,994.

My invention relates to temperature measuring devices and particularly to pyrometer tubes.

An object of my invention is to provide a structure for a pyrometer tube that shall permit of the tube being quickly inserted in and withdrawn from the chamber of a furnace without danger of cracking or breaking.

Another object of my invention is to provide a unitary pyrometer tube that shall embody a gas tight inner refractory portion and a heat-insulating or heat-equalizing outer ceramic portion.

In practicing my invention I provide an inner tube which is composed either of a highly refractory metal or of porcelain which has been made and fired in the usual manner, the inner tube being surrounded or covered by a relatively thick coating of a highly refractory cement consisting of a high temperature clay and fused alumina.

In the single sheet of drawings,

Figure 1 is a view, in longitudinal section, of a device embodying my invention, and, 25 Fig. 2 is a view, in vertical lateral section, of a furnace with which is associated the device embodying my invention.

It has heretofore been found necessary to use a substantially stationary tube supported 30 by and in one of the walls of a furnace and extending therethrough into the furnace chamber, this tube being of ordinary refractory material and of such diameter as to permit of fitting thereinto a smaller ceramic 35 tube within which is located the usual thermocouple, by means of which, when used in combination with suitable indicating instruments the temperature of the furnace chamber may be measured. It has been found 40 necessary to insert and withdraw the inner tube very slowly in order to avoid breaking it because of the change in temperature to which it is subjected.

Referring more particularly to Fig. 1 of 45 the drawing I have there illustrated a pyrometer tube assembly 11 embodying an inner tube 12 which is made either of a highly refractory metal such as nickel, or of porcelain which has been fired at a suitable temperature 50 of about 2000° F. I provide an outer

cement coating or tube 13 therearound, comprising a mixture of comminuted fused alumina, a high temperature clay, and a small amount of a suitable binder such as dextrine. I prefer to use a mixture of approximately 55 30% of high temperature clay and approximately 70% of fused alumina, although I desire it to be understood that this proportion may be departed from to a certain extent. Enough binder is added to the finely divided 60 mixed dry clay and fused alumina to make a relatively moist mixture of the general consistency of heavy cream.

The tube 12 is then dipped into this moistened cement mixture a sufficient number of 65 times to provide a relatively heavy closely adherent coating around the exterior of the porcelain tube. It may be necessary to permit each coating to dry for a short period 70 of time in air before another dipping in order that it may be possible to provide a coating that shall be of even thickness over the entire area thereof.

As shown in the drawing one end of the tube is closed. While I have indicated that 75 the wall-thickness of the inner tube is slightly less than that of the outer tube, I do not desire to be limited thereto as the relative thicknesses of the wall are of no particular moment, except that both thicknesses should 80 be relatively large and I prefer that the radial thickness of the outer tube shall be not less than  $\frac{1}{4}$  inch, and I may make it two or three times this value.

After the plurality of coatings have been 85 permitted to dry in air I place the tube in a suitable furnace chamber operating at a temperature of not less than 2000°, and possibly up to 3000° F. The firing is continued until the inner tube 12 has been re-fused to a greater extent than occurred during its initial firing, if made of porcelain, the effect being that the inner tube is rendered substantially gastight. This is of importance in the case 90 of certain furnace operations in which there might be a tendency for the atmosphere in the chamber to be of an oxidizing character and to penetrate the walls of the tube.

If the inner tube is of a highly refractory 95 metal, such as nickel, the firing temperature 100

must be such that the nickel or other metal is not softened or otherwise affected in a manner to reduce the cementing action of the mixture of fused alumina and high temperature clay. It may be noted here that the term "high temperature clay" is a generic one and is here used to cover any clay that will withstand relatively high temperatures, irrespective of the composition thereof. This coating or outer tube will adhere closely to the inner tube being cemented thereto by its own adhesive action and will withstand or resist the action of slag, acid, or oxidizing atmosphere. It is made thick enough to have a heat-equalizing effect and is thus able to withstand sudden relatively great changes in temperature without cracking or breaking.

Fig. 2 illustrates the use of the pyrometer tube embodying my invention. A furnace is indicated generally by 14 and comprises a plurality of walls of heat-insulating and high temperature resisting bricks or blocks surrounding a furnace chamber 15. An opening 16 is provided in one of the walls of the furnace of such size as to receive the pyrometer tube 11. A thermocouple 17 is located within the inner tube 12, the joint thereof being located within the furnace chamber 15, the tube 11 extending sufficiently far into the furnace chamber to subject the thermocouple joint to the operating temperature of the chamber. The two wires of the thermocouple are connected to a suitable temperature indicating means usually employed in the art, by means of which the operating temperature of the furnace chamber may be determined.

I have found, by actual tests, that it is possible to quickly insert a composite pyrometer tube of the kind embodying my invention through the opening 16 in a furnace wall, without the tube cracking or breaking. I have found it possible also to quickly remove such a pyrometer tube from the furnace structure without its cracking or breaking, even though the temperature of the furnace be well above 2000° F. I attribute this to the relatively thick protective and heat-equalizing coating on the outside of the inner refractory tube, which protective coating or tubing is made of such thickness and of such material as to permit of its being subjected to relatively rapid and large temperature changes without overstressing the walls of the tube.

Various modifications may be made in the device embodying my invention without departing from the spirit and scope thereof, and I desire therefore, that only such limitations shall be placed theron as are imposed by the prior art or are set forth in the appended claims.

I claim as my invention:

1. As a new article of manufacture of the class described, a fired unitary refractory

composite pyrometer tube structure comprising an inner tube of refractory material and an outer heat-equalizing tube of refractory ceramic material therearound and intimately bonded thereto by firing.

2. As a new article of manufacture, a fired composite unitary pyrometer tube structure comprising an inner tube of refractory material and an outer closely adherent coating of a highly refractory material comprising fused alumina, clay, and a binder, said coating and tube being intimately bonded by firing the coated tube.

3. As a new article of manufacture, a fired composite unitary pyrometer tube structure comprising an inner tube of gas proof porcelain, and an outer closely adherent coating, of substantially the same or greater thickness as the inner tube, and comprising fused alumina, a high temperature clay and a binder, said coating and tube being intimately bonded by firing the coated tube.

4. As a new article of manufacture, a fired composite unitary pyrometer tube comprising a doubly fired inner tube of gas proof porcelain and a singly fired outer closely-adherent heat equalizing covering therearound comprising fused alumina, a high temperature clay and a binder, said covering and tube being intimately bonded by jointly firing the tube and covering.

5. As a new article of manufacture, a fired composite unitary pyrometer tube comprising a doubly fired inner tube of porcelain and a singly fired outer closely-adherent covering therearound comprising a mixture of approximately 30% fused alumina, and approximately 70% of a high temperature clay, said covering and tube being intimately bonded by jointly firing the tube and covering.

In testimony whereof, I have hereunto subscribed my name this 10th day of October, 1927.

FRANK C. SIMMS.

110

115

120

125

130